

# UNITED STATES PATENT OFFICE.

CHARLES M. UPHAM, OF STOUGHTON, MASSACHUSETTS.

## SURFACING MATERIAL FOR ROADS.

1,240,269.

Specification of Letters Patent. Patented Sept. 18, 1917.

No Drawing.

Application filed June 28, 1912. Serial No. 706,517.

To all whom it may concern:

Be it known that I, CHARLES M. UPHAM, of Stoughton, in the county of Norfolk, and in the State of Massachusetts, have invented 5 a certain new and useful Improvement in Surfacing Material for Roads, and do hereby declare that the following is a full, clear, and exact description thereof.

The object of my invention has been to 10 provide an improved surfacing material for roads which shall have, among others, the following advantages:

That it can be made of any natural aggregate, so long as it does not contain too large 15 stones, and can, therefore, use any earthy material or mineral matter which may be found available nearest the location of the road upon which it has to be laid; that it shall not become soft and spongy during 20 hot weather, and shall not become brittle in cold weather, and that it shall, therefore, be cheap and durable; and to such ends my invention consists in the surfacing material 25 for roads hereinafter specified.

25 While I have illustrated my invention by the best embodiment thereof known to me, such embodiment is to be regarded as typical only of many possible embodiments, and 30 definite statements are to be regarded as illustrative only, and capable of wide variation.

My invention relates to that class of roads in which a bituminous surface material is used having a natural aggregate. Such 35 roads consist of a bituminous binder and an earthy or mineral material mixed therewith and called an "aggregate".

I have desired to provide a surfacing material in which any available earthy or mineral material could be used as the aggregate; this enables the material of an old 40 road, being made over, to be used, or rock, sand or soil in the immediate neighborhood to be used. Prior to my invention, so far 45 as known to me, all road surfaces using a natural aggregate with a bituminous binder becomes soft and spongy in hot weather and thus increase the effort to draw a load thereon. Moreover, by softening in this 50 way, the tendency of particles of the road to be torn away from the road bed is greatly increased. Moreover, such prior roads become brittle at lower temperatures and tend to disintegrate.

55 According to my invention, I use a binder with a relatively high melting point and

relatively low degree of penetration. The high melting point may be obtained by using a bitumen having suitable characteristics, that is, one which has, for instance, 60 had either dry steam or air blown through it while in a fluid condition. This makes it less susceptible to temperature changes, that is, it does not become brittle even at low temperatures. The quality of resistance to 65 high temperatures or "the low penetration" is obtained by greater distillation, that is, by distilling off the lighter products. This process also increases the degree of the melting point. The "penetration" refers to the 70 extent to which an object, such as a needle of a given size, will penetrate the bitumen under a given weight in a given time. As a specific instance of a binder which I find to work advantageously, one having a melting point of 150° F., and a penetration, 75 when measured with a standard penetrometer (Dow), fitted with a No. 2 needle weighted with a 100 gram weight applied for five seconds with the bitumen maintained at 80 77°, shall not be more than 55°. The figures given in this specific instance are only given for the purpose of stating a specific example, and it is to be understood that they are capable of very wide variation. 85

In making a surfacing material, I mix with whatever available earthy or mineral material there may be, a suitable quantity of the said binder, preferably depending upon the binder to give the pavement 90 stability, and not depending upon the form of the aggregate for that purpose.

I find that if the pavement is not sufficiently dense, owing to the fact that the aggregate is too coarse, I can substantially 95 increase the density by the addition of finer material, such as dust, silt, pulverized clay, soil or similar very fine material. The proportion of this fine material may be as great as two-thirds of the proportion of the 100 aggregate.

In building a road, using my invention, the sub-grade of the road is shaped and compacted by any desirable means, so as to present a surface free from depressions 105 and parallel to the surface of the finished road. My said surfacing material is then spread upon this prepared sub-base to the desired depth, and preferably rolled and compacted until the surface is free from 110 depressions and is properly shaped.

Before the final rolling, a layer of stone,

dust, screenings, mineral chips, slag, or other mineral grit is preferably spread upon and rolled into the surfacing. This gives the surfacing a "tooth" and prevents it becoming slippery.

I claim:

1. A surfacing material for roads comprising a bitumen having a melting point of substantially  $150^{\circ}$  F. and a penetration not substantially more than  $55^{\circ}$  measured with a Dow penetrometer with 100 gram weight at a temperature of  $77^{\circ}$  F.
2. A surfacing material for roads comprising a bitumen having a melting point of substantially  $150^{\circ}$  F. and a penetration not substantially more than  $55^{\circ}$  measured with a Dow penetrometer with 100 gram

weight at a temperature of  $77^{\circ}$  F., and a natural aggregate.

3. A surfacing material for roads comprising a bitumen having a melting point of substantially  $150^{\circ}$  F. and a penetration not substantially more than  $55^{\circ}$  measured with a Dow penetrometer with 100 gram weight at a temperature of  $77^{\circ}$  F. and a natural aggregate comprising a large proportion of fine material mixed with larger material.

In testimony that I claim the foregoing I have hereunto set my hand.

CHARLES M. UPHAM.

Witnesses:

FRANCIS A. ROSELL,  
A. M. GORMAN.